

Patented Feb. 23, 1926.

1,574,374

# UNITED STATES PATENT OFFICE.

WILLIAM J. DIEDERICHS AND ANSON HAYES, OF AMES, IOWA.

## PROCESS FOR TREATING IRON.

No Drawing. Application filed August 21, 1922, Serial No. 583,370. Renewed August 28, 1925.

To all whom it may concern:

Be it known that we, WILLIAM J. DIEDERICHS and ANSON HAYES, each a citizen of the United States of America, and residents of Ames, Story County, Iowa, have invented a new and useful Process for Treating Iron, of which the following is a specification.

The object of this invention is to provide 10 a new and improved process for treating white cast iron, whereby an iron is produced practically duplicating the properties of commercial malleable iron, and in a much shorter time than now required in the 15 ordinary malleableizing process.

A further object of this invention is to shorten the time required for producing malleable iron.

These and other objects of the invention 20 will be more clearly described in the specification and pointed out in the appended claims.

Any suitable type or form of furnace or so-called annealing oven may be employed 25 in carrying out our improved process, and may be heated by any of the well known fuels such as gas, oil, or powdered coal burned in connection with air; or the heat may be secured electrically or by a combination of combustion and electricity, or 30 in any other manner that may be desired so long as the desired temperatures and atmospheres are secured.

The iron used in this process is known as 35 white cast iron such as is used in making malleable castings. This white cast iron differs principally from ordinary gray iron in that while both contain carbon the white cast iron contains the carbon wholly or principally in the form of carbide of iron represented by the formula  $Fe_3C$ , while gray cast iron contains the carbon to a greater degree in the form of graphite or graphitic carbon. 40 It is well known that ordinarily in making malleable castings the white iron is packed with some oxidizing or packing material in sealed boxes or pots which are loaded into the furnace while the furnace is cold and the furnace is then gradually 45 raised to a temperature of between 800 and 850 degrees centigrade and maintained at that temperature for approximately sixty hours, after which the furnace is gradually cooled, the whole process requiring seven to 50 nine days of continuous operation. In the making of malleable castings the iron car-

bid is changed mainly to iron and temper carbon or graphite, the resulting iron usually having a lower tensile strength than the white cast iron from which it was made, 60 but it will bend or stretch to an appreciable degree, which is not true of the white cast iron.

In carrying out our improved process we use the white cast iron just as in the process above described, but we employ a very different and much shorter process, which may involve higher temperatures at times. By carrying this process entirely through to its conclusion as hereinafter set forth, we 65 obtain a product fully as characteristic and practically duplicating all the properties of malleable iron produced by the now common and well known methods, but in a much shorter time. 75

In carrying out our improved process we do not necessarily pack the white iron castings as in the ordinary malleableizing process, although that may be done at times if desired. By omitting it considerable time is 80 saved. When the packing is omitted the white iron castings may be supported in any suitable manner in the furnace to prevent sagging and warping under intense heat. The process consists in heating for any 85 length of time, raising the temperature of the white iron castings with convenient rapidity, either rapidly or slowly, to any point between the critical temperature of the material (about 740 degrees centigrade) 90

and the point of incipient fusion and holding at the chosen higher temperature for a period of fifteen minutes to five hours, or more. The actual time required will depend upon the temperature chosen, lower temperatures requiring longer times, and upon the chemical composition of the white iron being treated. In any case it is only desired to maintain the higher temperature until the massive cementite is practically all absorbed in the solid solution. We are satisfied that in most instances it would avail little to hold at the higher temperature for a longer period than about five hours, since practically all of the desirable change would have occurred in that time, especially if the high temperature employed is above 1650 degrees F.; and that holding for longer periods would result only in a waste of time without corresponding benefit. If a high 100 temperature of less than 1650 degrees F. is used the time required to practically com-

plete the absorption of massive cementite into the solid solution will be very materially increased. The material is then cooled rapidly or slowly to a temperature either in the neighborhood of the critical temperature, either within or outside of the heating furnace. These operations may be repeated for any desired number of repetitions, that is to say, the material may be alternately heated to a point above the critical temperature and cooled to a temperature in the neighborhood of or slightly below the critical. The iron may be cooled in the furnace or in any suitable manner. It has been demonstrated by experiment that the resultant product is an iron possessing considerably greater strength than the white iron castings and also having a considerable degree of ductility. The number of repetitions or alternate heatings and coolings, as well as the rates of heating and cooling, may be varied in accordance with the properties desired in the product.

An additional or final step is added which characterizes the resultant product as malleable iron. The operations are carried out as above described, that is either a single heating to a point above the critical temperature for a period of fifteen minutes to five hours or more followed by a cooling to a point in the neighborhood of the critical, or repetitions of such alternate heating and cooling; and the final step consists in making the final cooling extremely slowly. This results in a product duplicating approximately the properties of commercial malleable iron, that is having a tensile strength of from 44000 to 53000 pounds per square inch and an elongation or ability to stretch of fifteen per cent or more, in two inches. The process is much shorter than that now carried out to obtain commercial malleable iron.

Our experiments show that the treatment of the iron as described results in castings possessing a tensile strength, of from about 44000 to 53000 pounds per square inch or more and an elongation or ability to stretch of ten per cent, or more, in two inches, a material closely approximating the properties of commercial malleable iron, as above set forth.

We have also found that by a combination of the high temperature followed by a repetition of alternate heating and cooling; or vice versa, that is alternate heating and cooling, with a heating to higher temperature following or interposed, we obtain a resulting material of the same properties as that obtained by either one of the methods individually.

As a concrete example of what we have obtained in our experiments, we recite one instance by way of illustration only. A bar of white iron was heated to 1000 degrees centigrade, with the furnace, held at that

temperature for one hour, cooled to 850 degrees with the furnace (requiring about two hours); held at that temperature for six hours, and then allowed to cool very slowly, at the rate of somewhat less than five degrees centigrade per hour. The resulting material possessed a tensile strength of 49200 pounds per square inch and an elongation of 16.5 per cent in two inches. We believe that the result attained in this instance is due to the combined high temperature (for a short period of time) and the extremely slow cooling, whereby we obtain in a much shorter time than now required, a product possessing the characteristics of commercial malleable iron.

Likewise by way of illustration, we heated white cast iron bars beyond the critical temperature, in fact to about 850 degrees centigrade, and cooled them successively to a point in the neighborhood of or below the critical temperature, for eight successive repetitions, then heated again and cooled extremely slowly, at the rate of about or somewhat less than five degrees centigrade per hour, and obtained a product having 46000 pounds strength per square inch and an elongation of 17.5 per cent.

The overall time required for the experiments of which the above are two concrete examples was in the neighborhood of forty-five hours, but in these experiments, as a precautionary measure, the slow cooling was continued over a much greater range than necessary, so that it is certain this overall time can be materially reduced.

Referring to the final cooling of the castings at an extremely slow rate, we have found that a cooling at the rate of about or somewhat less than five degrees centigrade per hour gives the best result, but a somewhat more rapid cooling may be employed without departing from our invention, but with rather less of the characteristic malleable properties in the resultant product.

When speaking of the critical temperature of the material, the fact should be borne in mind, which is well known in metallurgy, that the critical temperature can be, and is, undercooled by a rapid cooling, and therefore will be reduced by heating to a temperature above the critical and cooling fairly rapidly; so that in thereafter heating to the critical temperature, it is obvious that a lower actual temperature will be involved. The language of this specification and the appended claims is used with this fact in mind and should be so construed.

We claim as our invention—

1. The process for the heat treatment of castings from white cast iron which consists in (1) subjecting of the casting to a temperature above the critical temperature of the material for a period of from fifteen minutes to five hours or more but only until

the iron carbide present is practically all absorbed in the solid solution, which means that in irons of commercial composition the combined carbon is reduced to approximately nine-tenths of one percent; (2) the cooling of the casting to a lower temperature in the neighborhood of the critical temperature; and (3) the cooling of the casting to room temperature.

13 2. The process for the heat treatment of castings from white cast iron which consists in (1) subjecting of the casting to a temperature above the critical temperature of the material for such time only that the iron carbide present is practically all absorbed in the solid solution, or in other words that in irons of commercial composition the combined carbon is reduced to substantially nine-tenths of one percent, this requiring 20 from fifteen minutes to five hours or more; (2) the cooling of the casting to a temperature in the neighborhood of the critical temperature; and (3) the cooling of the casting at an extremely slow rate.

25 3. The process for the heat treatment of castings from white cast iron which consists in (1) subjecting of the casting to a temperature considerably above the critical temperature of the material for a period of 30 from fifteen minutes to five hours, or more, until the iron carbide present is practically all absorbed in the solid solution or in other words until in irons of commercial composition the combined carbon is reduced 35 to substantially nine-tenths of one percent; (2) the cooling of the casting to a temperature in the neighborhood of the critical temperature; and (3) the cooling of the casting to a still lower point.

40 4. The process for the heat treatment of castings from white cast iron which consists in (1) the subjecting of the casting to a temperature above the critical temperature of the material, (2) the cooling of the casting to a temperature in the neighborhood of the critical temperature and (3) a repetition of the above named steps, alternately.

45 5. The process for the heat treatment of castings from white cast iron which consists in (1) the subjecting of the casting to a temperature above the critical temperature of the material, (2) the cooling of the casting to a temperature in the neighborhood of

the critical temperature, (3) alternate repetition of the above named steps and (4) a final heating to a point above the critical temperature followed by an extremely slow cooling, at the rate of about five degrees centigrade per hour.

60 6. The process for the heat treatment of castings from white cast iron which consists in (1) the subjecting of the casting to a heating considerably above the critical temperature of the material, (2) the cooling 65 of the casting to a temperature in the neighborhood of the critical temperature, (3) the heating of the casting to a temperature above the critical temperature, (4) the cooling of the casting to a temperature in 70 the neighborhood of the critical temperature (5) the repeating of steps (3) and (4) alternately and (6) permitting the casting to cool to a still lower temperature.

75 7. The process for the heat treatment of castings from white cast iron which consists in (1) the subjecting of the casting to a heating in the neighborhood of 1000 degrees centigrade more or less for a period ranging from about fifteen minutes to five hours or more, (2) the cooling of the casting to a temperature of between about 850 degrees and about 740 degrees centigrade, (3) the maintaining of the casting at about the temperature recited in step (2) for a 80 time sufficient to allow a suitable approach to chemical equilibrium of the constituents, and (4) the cooling of the casting at a slow rate of about five degrees centigrade per 85 hour.

90 8. The process for the heat treatment of castings from white cast iron which consists in (1) the subjecting of the casting to a heating in the neighborhood of 1000 degrees centigrade more or less for a period ranging from about fifteen minutes to five hours or more, (2) the cooling of the casting to a temperature between about 850 degrees and about 740 degrees centigrade, (3) the maintaining of such temperature 95 for a time sufficient to allow a suitable approach to chemical equilibrium of the constituents, and (4) the cooling of the casting.

95 Signed at Des Moines, in the County of Polk and State of Iowa, this 18th day of August, 1922.

WILLIAM J. DIEDERICHS.  
ANSON HAYES.